# EUROPEAN PATENT SPECIFICATION

(11) **EP 0 007 247 B1**
(45) Date of publication and mention of the grant of the patent: **24.11.1982**
(21) Application number: 79301418.4
(22) Date of filing: 17.07.1979
(51) Int. Cl.: C10J 3/00, C10J 3/54

(54) **A process for the catalytic gasification of carbonaceous materials**
Verfahren zur katalytischen Vergasung von kohlenstoffhaltigen Brennstoffen
Procédé pour la gazéification catalytique de matières carbonées

(30) Priority: 17.07.1978 US 925664
(43) Date of publication of application: 23.01.1980
(73) Proprietor: EXXON RESEARCH AND ENGINEERING COMPANY, Florham Park, New Jersey 07932-0390 (US)
(72) Inventor: Lang, Robert Joseph, Baytown, Texas (US); Pabst, Joanne Keel, Crosby, Texas (US)
(74) Representative: Somers, Harold Arnold

## Description

The present invention relates to a process for the catalytic gasification of carbonaceous materials such as oils, petroleum residua, coals and the like, carried out in the presence of alkali metal-containing catalysts.

It has long been recognised that certain alkali metal compounds can be employed to catalyze the gasification of carbonaceous materials such as coal and other carbonaceous solids. Studies have shown that potassium carbonate, sodium carbonate, cesium carbonate and lithium carbonate will substantially accelerate the rate at which steam, hydrogen, carbon dioxide, oxygen and the like react with bitiminous coal, subbituminous coal, lignite, petroleum coke, organic waste materials and similar carbonaceous solids to form methane, carbon monoxide, hydrogen, carbon dioxide and other gaseous products. Other alkali metal salts such as alkali metal chlorides, however, have a low catalytic activity when compared to that of the corresponding carbonate. Because of the relatively high cost of cesium carbonate and the low effectiveness of lithium and sodium carbonates, most of the experimental work in this area which has been carried out in the past has been directed towards the use of potassium carbonate.

In addition to utilizing individual alkali metal salts as a catalyst for the gasification of a carbonaceous material, it has been proposed to utilize mixtures of alkali metal salts. When such mixtures of alkali metal salts are used to promote the gasification of a carbonaceous feed material, it is expected that the mixture will accelerate the gasification reactions less than if an equivalent amount of the more active alkali metal compound is used alone and more than if an equivalent amount of the less active alkali metal salt is employed.

In gasification processes using alkali metal-containing catalysts, the cost of the catalyst is a significant factor in determining the overall cost of the product gas. Potassium carbonate is relatively expensive.

The costs of other alkali metal compounds such as potassium chloride, potassium sulfate, sodium carbonate, sodium chloride and sodium sulfate are substantially cheaper than potassium carbonate but these compounds exhibit only a fraction of the catalytic activity exhibited by potassium carbonate. It would be highly desirable if the compounds mentioned above and other more abundant, less expensive potassium and sodium compounds could be effectively used as gasification catalysts thereby substantially decreasing the initial investment required in the catalyst and obviating the need for expensive secondary recovery techniques to decrease the amount of makeup alkali compounds that would otherwise be required to maintain the catalyst inventory at the required level.

It has now been found that catalyst costs incurred during the gasification of oils, petroleum residua, bituminous coal, subbituminous coal, lignite, organic waste material, petroleum coke, and other carbonaceous feed materials can be significantly reduced while at the same time obtaining unexpectedly high gasification rates by employing mixtures of inexpensive potassium compounds and sodium or lithium compounds as the catalyst, and according to the invention, there is provided a process for the catalytic gasification of a carbonaceous feed material in a rection zone under gasification conditions in the presence of a catalyst comprising a potassium salt, wherein the process comprises introducing into the reaction zone: (a) a potassium salt of an organic or inorganic acid having an ionization constant exceeding 10-³ at 25°C; and (b) a sufficient quantity to activate the potassium salt of a sodium or lithium compound which is either a salt of a weak acid or a salt of a strong acid that is converted to a salt of a weak acid at the gasification conditions of the gasification process.

The potassium salt and sodium or lithium compounds introduced into the reaction zone may be present in concentrations sufficient to yield a sodium or lithium to potassium atomic ratio of at least 0.25.

The potassium salt introduced into the reaction zone may be, e.g. potassium chloride, and sodium compound is preferably present in concentrations sufficient to yield an atomic ratio of sodium to potassium of at least 1.0. Laboratory tests have shown that when mixtures of coal, potassium chloride or potassium sulfate, and sodium carbonate or sodium sulfate are injected into a reaction zone and the coal is subsequently gasified, surprisingly high gasification rates are obtained. These gasification rates are substantially higher than expected based on the low activity of the individual potassium and sodium compounds relative to that of potassium carbonate. This is a significant and unexpected discovery since the observed gasification rates are high enough to enable mixtures of these inexpensive potassium and sodium salts to be used as gasification catalysts in lieu of the substantially more expensive potassium carbonate. Because of the quantities in which catalysts are required in catalytic gasification operations, the overall savings made possible in a large gasification plant by the invention may be quite substantial.

In general, unexpectedly high gasification rates will be obtained when a carbonaceous feed material is introduced into a reaction zone along with a mixture of a potassium compound having a relatively poor catalytic activity as compared to that of potassium carbonate and a sodium or lithium compound selected from the group consisting of a weak acid salt of sodium or lithium and a strong acid salt of sodium or lithium that is converted to a weak acid salt in the reaction zone at reaction conditions, and the carbonaceous material is subsequently gasified. For mixtures of certain relatively noncatalytic potassium and sodium compounds, the gasification rate obtained will be nearly as great as the rate obtained when potassium carbonate alone is introduced into the reaction zone with the feed material in an amount that yields the same alkali metal-to-carbon atomic ratio as that of the mixture. Evidently, the sodium or lithium compound activates the poorly catalytic potassium compound thereby producing a substantial catalytic effect on the gasification rate of the carbonaceous feed material.

In accordance with the invention, the use of catalysts containing mixtures of inexpensive potassium and sodium or lithium compounds reduces the initial catalyst cost and the cost of makeup catalyst and at the same time permits the attainment of high gasification rates. The use of such mixtures also obviates the need for expensive secondary catalyst recovery procedures. As a result, the invention makes possible substantial savings in gasification operations and permits the generation of product gases at significantly lower cost than would normally otherwise be the case.

### BRIEF DESCRIPTION OF THE DRAWINGS

Figure 1 in the drawing is a schematic flow diagram of a process for the gasification of coal carried out in accordance with the invention;
Figure 2 is a plot illustrating that unexpectedly high gasification rates are obtained by using a mixture of potassium sulfate and sodium carbonate which is equimolar in potassium and sodium to catalyze the gasification of a carbonaceous material;
Figure 3 is a plot illustrating that unexpectedly high gasification rates are obtained by using a mixture of potassium sulfate and sodium sulfate which is equimolar in potassium and sodium to catalyze the gasification of a carbonaceous material;
Figure 4 is a plot illustrating that unexpectedly high gasification rates are obtained by using a mixture of potassium sulfate and sodium chloride which is equimolar in potassium and sodium to catalyze the gasification of a carbonaceous material;
Figure 5 is a plot illustrating that unexpectedly high gasification rates are obtained by using a mixture of potassium sulfate and sodium nitrate which is equimolar in potassium and sodium to catalyze the gasification of a carbonaceous material;
Figure 6 is a plot illustrating that unexpectedly high gasification rates are obtained by using a mixture of potassium chloride and sodium carbonate which is equimolar in potassium and sodium to catalyze the gasification of a carbonaceous material;
Figure 7 is a plot illustrating that unexpectedly high gasification rates are obtained by using a mixture of potassium chloride and sodium sulfate which is equimolar in potassium and sodium to catalyze the gasification of a carbonaceous material;
Figure 8 is a plot illustrating that unexpectedly high gasification rates are obtained by using a mixture of potassium and lithium to catalyze the gasification of a carbonaceous material;
Figure 9 is a plot illustrating that the addition of small amounts of various sodium salts will activate relatively noncatalytic potassium. sulfate thereby rapidly increasing the gasification rate" of a carbonaceous material; and
Figure 10 is a plot illustrating that the catalytic gasification activity of relatively noncatalytic potassium chloride can be substantially increased by adding sodium carbonate in an amount sufficient to yield a sodium-to-potassium mole ratio of 1.0 or greater.

### DESCRIPTION OF THE

### PREFERRED EMBODIMENTS

The process depicted in Figure 1 is one for the gasification of bituminous coal, subbituminous coal, lignite, organic waste materials or similar carbonaceous solids in the presence of added sodium and potassium compounds. It will be understood that the invention is not restricted to this particular gasification process and instead may be employed in any of a wide variety of fixed bed, moving bed and fluidized bed gasification operations in which alkali metal compounds are used to promote the reaction of steam, hydrogen, carbon dioxide, or a similar gasification agent with carbonaceous feed materials and a char, coke or other solid product containing alkali metal residues is recovered. Many such operations have been described in the technical literature and will be familiar to those skilled in the art.

In the process shown, a solid carbonaceous feed material such as bituminous coal, subbituminous coal, lignite or the like, which has been crushed and screened to a particle size of about 8 mesh or smaller on the U.S. Sieve Series Scale is fed into the system through line 10 from a coal preparation plant or storage facility which is not shown in the drawing. The solids introduced through line 10 are fed into a hopper or similar vessel 12 from which they are passed through line 13 into a feed preparation zone 14. The feed preparation zone shown includes a screw conveyor or similar device, not shown in the drawing, which is powered by a motor 16, a series of spray nozzles or the like 17 for the spraying of a solution of soluble alkali metal compounds introduced through line 18 onto the solids as they are moved through the preparation zone by the conveyor, and nozzles or the like 19 for the introduction of steam from line 20 into the preparation zone to heat the solids and drive off moisture. The alkali metal solution fed through line 18 is prepared by introducing soluble sodium and potassium salts or other sodium and potassium compounds into mixing vessel 21 as indicated by lines 22 and 23, respectively and dissolving these in water or other suitable solvent solution admitted through line 24. Alkali metal solution recycled from the catalyst recovery zone through line 25 as described hereafter may also be used. Steam is withdrawn from the preparation zone 14 through line 28 and will normally be passed to a condenser or heat exchanger not shown for the recovery of heat and condensate which can be used as makeup water or the like.

The potassium compound introduced into mixing vessel 21 through line 23 will normally be an inexpensive compound which has a relatively poor catalytic activity as compared to that of potassium carbonate. "Relatively poor catalystic activity as compared to that of potassium carbonate" as used herein refers to a gasification rate obtained from gasifying a carbonaceous material in the presence of a sufficient amount of potassium compound to yield an atomic ratio of potassium cations-to-carbon atoms of about .03 or greater that is about one-half or less that of the rate obtainable by gasifying the same material in the presence of an equivalent amount of potassium carbonate. Examples of such potassium compounds include potassium chloride, potassium sulfate, and similar potassium salts of a strong acid. "Strong acid" as used herein refers to an organic or inorganic acid having an Ionization constant greater than about 1 x 10-³ at 25°C.

The sodium compound introduced into mixing vessel 21 through line 22 will normally be either a sodium salt of a weak acid or a sodium salt of a strong acid that is converted, either temporarily or permanently, into a weak acid salt of sodium when subjected to gasification conditions in the presence of the potassium compound. "Weak acid" as used herein refers to an organic or inorganic acid having an ionization constant less than about 1 x 10-³ at 25°C. Examples of suitable sodium compounds that are salts of weak acids including sodium hydroxide, sodium carbonate; sodium bicarbonate, sodium sulfide, sodium oxalate, sodium acetate, and the like. Examples of sodium salts of strong acids that may be used in conjunction with potassium sulfate because they are temporarily or permanently converted to weak acid salts include sodium chloride, sodium sulfate and sodium nitrate. The actual sodium compound used will normally depend upon its availability, cost, degree of solubility and the potassium compound utilized.

It has been surprisingly found that when mixtures of the potassium and sodium compounds referred to above are injected into a catalytic gasification zone with a carbonaceous feed material which is subsequently gasified in the zone, gasification rates are obtained that are much higher than those that would normally be expected by one of ordinary skill in the art. Apparently, the poorly catalytic potassium compound is activated by the sodium compound thereby producing a substantial catalytic effect on the gasification rate of the carbonaceous feed material. Normally a concentration of the sodium compound sufficient to yield a sodium-to-potassium mole ratio of 1.0 will completely activate the potassium compound. In some mixtures, however, lesser amounts of the sodium compound may be used to activate the potassium compound without much activity loss.

The actual mechanism by which the sodium compound activates the potassium compound in the presence of the carbonaceous feed material and under gasification conditions is not fully understood. It is believed, however, that certain interactions between the compounds take place which eventually result in transforming the poorly catalytic strong acid salt of potassium into a catalytically active weak acid salt. For example, the following equations are believed to represent the reactions that take place when the potassium compound utilized is potassium sulfate and the sodium compound utilized is sodium carbonate. As can be seen in equations (1) and (2), the anion associated with the potassium compound and the anion associated with the sodium compound exchange with one another to produce K₂CO₃ and Na₂SO₄, which is reduced in the presence of carbon, hydrogen or carbon monoxide under gasification conditions to Na₂S. The Na₂S then undergoes an anion exchange with the K₂SO₄ to produce K₂S and additional Na₂SO₄, which also is reduced to Na₂S. The net results of these reactions is the conversion of the poorly catalytic K_{Z}SO₄, a strong acid salt of potassium into catalytically active K₂CO₃ and K₂S, weak acid salts of potassium. The Na₂S that is formed is also catalytically active and is believed to add to the overall resultant catalytic activity of the original combination. It is believed that the weak acid salts, K₂CO₃, K₂S and Na₂S, react with the acidic carbonaceous solids to form an alkali metal-char "salt", which is believed to be the active site in gasification. Thus, in the case where the potassium compound is K₂SO₄ and the sodium compound is Na₂CO₃, both the potassium and sodium cations end up catalyzing the gasification of the carbonaceous solids.

If the potassium compound is potassium sulfate and the sodium compound is sodium sulfate, the following equations are belived to represent the reactions that take place. In the above-illustrated case; an anion exchange cannot take place between K₂SO₄ and Na₂SO₄ since the anions are identical. It is theorized, however, that the strong acid salt Na₂SO₄ is reduced in the presence of carbon, carbon monoxide or hydrogen under gasification conditions to the weak acid salt Na₂S, which then undergoes an anion exchange with the K₂SO₄ to produce K₂S and Na₂SO₄. The Na₂SO₄ thus formed is also reduced in the presence of carbon, carbon monoxide or hydrogen to Na₂S. The net result of these reactions is the formation of catalytically active K_{z}S and Na_{z}S and therefore, like the example illustrated in equations (1) and (2) above, both the potassium and sodium cations end up catalyzing the gasification of the carbonaceous solids.

It is believed that equations (5) and (6) set forth below represent the mechanism by which potassium sulfate is activated by sodium chloride. As can be seen, the potassium and sodium compounds exchange anions thereby forming KCl and Na₂SO₄. The Na₂SO₄ is then reduced under gasification conditions and in the presence of carbon, hydrogen or carbon monoxide to Na₂S, which undergoes an anion exchange with KCI to yield catalytically active K₂S and catalytically inactive NaCI, one of the original reactants. Thus, unlike the examples illustrated in equations (1) through (4) above, only the potassium cations end up catalyzing the gasification reactions.

As stated previously, any weak acid salt of sodium may be used to activate the relatively noncatalytic potassium compound, however, only certain strong acid sodium salts will be effective for this purpose. In general, only strong acid salts of sodium that are either temporarily or permanently converted to weak acid sodium salts under gasification conditions and in the presence of the potassium compound to be activated can be utilized. The examples illustrated by equations (3) through (6) above represent two cases in which relatively noncatalytic K₂SO₄ is activated by a strong acid sodium salt that is converted into a weak acid salt. In the example illustrated by equations (3) and (4), the strong acid sodium salt Na₂SO₄ undergoes reduction and is thereby permanently converted to the weak acid salt Na_{Z}S. In the example illustrated by equations (5) and (6), the strong acid salt NaCl is converted to the weak acid salt Na2S in a two-step process. First the NaCl participates in an anion exchange with the K₂SO₄ to form the strong acid salt Na₂SO₄ which then undergoes reduction to Na₂S. The Na₂S, however, then exchanges anions with KCI to reform the strong acid salt NaCI. This example, therefore, represents a case where a strong acid sodium salt is only temporarily converted to a weak acid salt. An example of a strong acid salt or sodium which is neither temporarily nor permanently converted to a weak acid sodium salt under gasification conditions in the presence of K₂SO₄ and therefore will not activate K₂S0₄ is Na₃P0₄.

The total quantity of the sodium and potassium compounds used should normally be sufficient to provide a combined added alkali metal-to-carbon atomic ratio in excess of about .03:1. Generally speaking, from about 5% to about 50% by weight of sodium and potassium compounds, based on the coal or other carbonaceous feed material will be employed. From about 10% to about 35% by weight is generally preferred. The higher the mineral content of the feed material, the more sodium and potassium compounds that should normally be used.

Referring again to Figure 1, the feed solids which are impregnated with sodium and potassium compounds in feed preparation zone 14 are withdrawn through line 30 and passed to a feed hopper or similar vessel 31. From here they are discharged through a star wheel feeder or a similar device 32 in line 33 at an elevated pressure sufficient to permit their entrainment in a stream of steam, recycle product gas, inert gas or other carrier gas introduced into the system through line 34. The carrier gas and entrained solids are passed through line 35 into manifold 36 and fed through multiple feed lines 37 and nozzles, not shown in the drawing, into gasifier 38. In lieu of or in addition to hopper 31 and star wheel feeder 32, the feed system employed may include parallel lock hoppers, pressurized hoppers, aerated standpipes operated in series, or other apparatus for raising the input feed solid stream to the required pressure level.

Gasifier 38 comprises a refractory-lined vessel containing a fluidized bed of carbonaceous solids extending upward within the vessel above an internal grid or similar distribution device not shown in the drawing. The solids are maintained in the fluidized state within the gasifier by means of a mixture of steam and oxygen injected through bottom inlet line 39 and multiple nozzles 40 connected to manifold 41. Sufficient oxygen is added to the steam through line 42 to maintain the fluidized bed at a temperature within the range between about 649°C (1200⁰F) and about 1093°C (2000°F). The gasifier (gauge) pressure will normally be between about 7.031 kg/cm² (100 psig) and about 140.614 kg/cm² (2000 psig). Under these conditions, the added sodium and potassium compounds result in the production of an unexpected and substantial catalytic effect on the steam gasification reaction thereby resulting in the production of a gas composed primarily of hydrogen, carbon monoxide and carbon dioxide. Other reactions will also take place and some methane will normally be formed depending on the gasification conditions.

The gas leaving the fluidized bed in gasifier 38 passes through the upper section of the gasifier, which serves as a disengagement zone where particles too heavy to be entrained by the gas leaving the vessel are returned to the bed. If desired, this disengagement zone may include one or more cyclone separators or the like for removing relatively large particles from the gas. The gas withdrawn from the upper part of the gasifier through line 43 is passed to cyclone separator or similar device 44 for removal of larger fines. The overhead gas then passes through line 46 into a second separator 47 where smaller particles are removed. The gas from which the solids have been separated is taken overhead from separator 47 through line 48 and the fines are discharged downward through dip legs 45 and 49. These fines may be returned to the gasifier or passed to the catalyst recovery section of the process as discussed hereafter. After entrained solids have been separated from the raw product gas, the gas stream may be passed through suitable heat exchange equipment for the recovery of heat and subsequently passed downstream for further processing.

Char particles containing carbonaceous material, ash and alkali metal residues are continuously withdrawn through line 50 from the bottom of the fluidized bed in gasifier 38. The particles flow downward through line 50 counter current to a stream of steam or other elutriating gas introduced through line 51. Here a preliminary separation of solids based on differences in size and density takes place. The lighter particles containing a relatively large amount of carbonaceous material tend to be returned to the gasifier and the heavier particles having a relatively high content of ash and alkali metal residues continue downward through line 52 into fluidized bed withdrawal zone 53. Steam or other fluidizing gas is introduced into the bottom of the withdrawal zone through line 54 to maintain the bed in the fluidized state. Water may be introduced through line 55 in order to cool the particles and facilitate their further processing. The withdrawal rate is controlled by regulating the pressure within zone 53 by means of throttle valve 56 in overhead line 57. The gases from line 57 may be returned to the gasifier through line 58 or vented through valve 59. From vessel 53 the solid particles are passed through line 60 containing valve 61 into hopper 62. The char fines recovered from the raw product gas through dip legs 45 and 49 may be combined with the char particles withdrawn from the gasifier by passing the fines through line 63 into hopper 62.

The particles in hopper 62 will contain sodium and potassium residues composed of water-soluble and water-in-soluble sodium and potassium compounds. These particles are passed from hopper 62 through line 64 into catalyst recovery unit 65. The catalyst recovery unit will normally comprise a multistage countercurrent extraction system in which the particles containing the sodium and potassium residues are countercurrently contacted with water introduced through line 66. An aqueous solution of sodium and potassium compounds is recovered from the unit and may be recycled through lines 67 and 25 to the catalyst preparation unit or mixing vessel 21. Particles from which substantially all of the soluble sodium and potassium constituents have been extracted are withdrawn from the catalyst recovery unit through line 68. These solids will normally contain substantial quantities of sodium and potassium present in the form of sodium and potassium aluminosilicates and other water-insoluble compounds. These compounds are formed in part by the reaction with the ash in the coal and other feed material of sodium and potassium compounds added to catalyze the gasification reaction. In general, from about 15% to as much as 50% of the added alkali metal constituents will be converted into alkali metal aluminosilicates and other water-insoluble compounds. By employing a mixture of inexpensive potassium and sodium compounds in accordance with the process of the invention in lieu of the more expensive potassium carbonate and other previously known catalysts, the need to recover and reuse the sodium and potassium compounds tied up as water-insoluble alkali metal residues by expensive and sophisticated secondary recovery methods is obviated.

In the embodiment of the invention described above, the feed solids are impregnated with a solution containing a mixture of sodium and potassium compounds prior to their introduction into the gasifier 38. It will be understood that other methods of introducing the sodium and potassium compounds into the gasification zone may be utilized. For example, the compounds may be mixed in the solid state with the carbonaceous feed particles and the mixture may be subsequently passed into the gasifier. In some cases it may be desirable to introduce the feed solids, the sodium compound and the potassium compound through separate lines into gasifier 38. Other methods for separate introduction of the sodium and potassium compounds into this system will be apparent to those skilled in the art.

The nature and objects of the invention are further illustrated by the results of laboratory gasification studies which show that unexpectedly high gasification rates are obtained by utilizing certain combinations of sodium and potassium compounds, and lithium and potassium compounds as catalysts. In all of the tests, about 2 grams of Illinois No. 6 coal crushed to about 0.6-0.15 mm (between about 30 and about 100 mesh on the U.S. Sieve Series Scale) was mixed with varying amounts of finely divided alkali metal compounds and combinations of such compounds. The resultant mixture was then dampened with about one milliliter of distilled water and pyrolyzed for about 15 minutes at about 760°C (1400°F) in a retort under an inert nitrogen atmosphere. A portion of the resultant char, containing between about 0.2 and about 0.5 grams of carbon, was then steam-gasified at a temperature of about 704°C (1300°F) and essentially atmospheric pressure in a laboratory bench scale gasification unit. The gasification rate obtained for each char sample was determined. The char not gasified was ashed to determine the amount of carbon present and the alkali metal cation-to-carbon atomic ratio was then calculated. The results of these tests are set forth in Figures 2 through 10. In all cases the gasification rate is expressed as the conversion weighted average rate in percent of carbon present per hour over the interval of 0-90% carbon conversion.

Figure 2 sets forth the steam gasification rate data obtained from char impregnated with various concentrations of potassium carbonate, potassium sulfate, sodium carbonate and a mixture of potassium sulfate and sodium carbonate. It can be seen in Figure 2 that the relatively expensive potassium carbonate yielded much greater gasification rates than did the less expensive potassium sulfate and sodium carbonate and is therefore a much more active gasification catalyst than either of the latter two compounds.

The dashed line in Figure 2 represents the gasification rates that one of ordinary skill in the art would expect to observe if a mixture of sodium carbonate and potassium sulfate which is equimolar in sodium and potassium (moles Na/K=1.0) was used as a catalyst. The expected gasification rate for such a mixture that yields an atomic ratio of .066 alkali metal cations per carbon atom was calculated as follows. The observed rate of about 51 % carbon per hour for a concentration of sodium carbonate that yielded an atomic ratio of .066 sodium cations per carbon atom was added to the observed rate of about 9.0% carbon. per hour for a concentration of potassium sulfate that yielded an atomic ratio of .066 potassium cations per carbon atom and the resultant value of 60% carbon per hour was divided by 2 to yield the expected rate of 30% carbon per hour. This rate was then plotted against the atomic ratio of .066 cations per carbon atom where .033 of the cations were potassium cations and the other .033 were sodium cations. The expected gasification rates for mixtures of sodium carbonate and potassium sulfate that are equimolar in sodium and potassium but yield alkali metal cation-to-carbon atomic ratios of other values were calculated in a manner similar to that described above.

As can be seen in Figure 2, the actual gasification rates observed using mixtures of potassium sulfate and sodium carbonate were much greater than the expected rates represented by the dashed line and approached the rates obtainable with equivalent concentrations of potassium carbonate. The actual observed gasification rate of an atomic ratio of .µ66 potassium and sodium cations per carbon atom was 83% carbon per hour as compared to the 30% carbon per hour that was expected. Furthermore, the actual observed rate of 83% carbon per hour for the mixture at an atomic ratio of .066 potassium and sodium cations per carbon atom is much greater than the 9.0% per hour obtained for potassium sulfate at an atomic ratio of .066 potassium cations per carbon atom and is also greater than the 51% carbon per hour obtained for sodium carbonate at an atomic ratio of .066 sodium cations per carbon atom. In view of the foregoing, the gasification rates obtained using mixtures of potassium sulfate and sodium carbonate as a catalyst are surprising and unexpected.

The data set forth in Figures 3 through 5 indicate that surprisingly high gasification rates can also be obtained by utilizing potassium sulfate in combination with various sodium salts other than sodium carbonate. Figure 3 shows that unexpectedly high rates are obtained using mixtures of potassium sulfate and sodium sulfate that are equimolar in potassium and sodium as a gasification catalyst. Figure 5 makes a similar showing for mixtures of potassium sulfate and sodium nitrate and are equimolar in potassium and sodium. In both Figures the rates one of ordinary skill in the art would expect are represented by dashed lines and were calculated as discussed previously in reference to Figure 2. Figure 4 shows that surprisingly high gasification rates are obtained using mixtures of potassium sulfate and sodium chloride that are equimolar in potassium and sodium. In Figure 4 the gasification rates for potassium sulfate alone and for sodium chloride alone fall on the same line. This line, therefore, also represents the gasification rates that would be expected for mixtures of the two salts that are equimolar in potassium and sodium.

Figures 6 and 7 illustrate that catalysts comprised of a mixture of potassium chloride and one of various inexpensive sodium salts will yield higher than expected gasification rates when the catalyst concentration is above a certain value. Figure 6 shows that surprisingiy high rates are obtained when a mixture of potassium chloride and sodium carbonate that is equimolar in potassium and sodium is employed in sufficient concentrations to yield an atomic ratio greater than about .08 alkali metal cations per carbon atom. Figure 7 makes a similar showing for a mixture of potassium chloride and sodium sulfate that is equimolar in potassium and sodium. As in previous Figures, the expected gasification rates are represented by a dashed line and were calculated as described in reference to Figure 2.

Figure 8 illustrates that a catalyst comprised of a mixture of a relatively noncatalytic potassium salt and a lithium salt - in lieu of a sodium salt - will also yield unexpectedly high gasification rates. It can be seen in Figure 8 that surprisingly high gasification rates are obtained when char is gasified in the presence of a mixture of potassium sulfate and lithium sulfate that is equimolar in potassium and lithium. As in prior Figures, the dashed line represents the gasification rate that would be expected by one of ordinary skill in the art.

Figure 9 shows the gasification rates obtained when Illinois No. 6 coal char was gasified in the presence of catalysts comprised of mixtures of potassium sulfate and varying amounts of either sodium carbonate, sodium sulfate or sodium chloride. In all cases the potassium sulfate was present in quantities such that the atomic ratio of potassium cations- to-carbon atoms ranged between about .051 and about .057. The amount of the particular sodium salt present was varied over a range such that the ratio of sodium cations to potassium cations present per carbon atom ranged from .25 to 1.0. This ratio (Na/K) is indicated next to each point plotted in the Figure. For comparison purposes, the rate of 8% carbon per hour obtained for the use of potassium sulfate alone (Na/K=0) is also shown in the Figure. It can be seen from the plotted data that for each combination of potassium sulfate and one of the three sodium salts, the presence of only a small amount of the sodium salt (Na/K=.25) resulted in a sharp increase in the gasification rate over that for a zero concentration of the sodium salt. The gasification rate continued to increase as the amount of the sodium salt in the mixture was increased up to a sodium-to-potassium atomic .ratio of 1.0.

Figure 10 is a plot similar to that of Figure 9 except that the gasification rates plotted are for a catalyst comprised of a mixture of potassium chloride and varying amounts of sodium carbonate. For comparison purposes, the rate of 18% carbon per hour for the use of potassium chloride alone (Na/K-0) is also shown in the Figure. As can be seen in the Figure, small amounts of the sodium carbonate (Na/K=.26 to .49) do not substantially increase the gasification rate. It is only when the amount of sodium carbonate in the mixture is sufficient to provide a sodium-to-potassium atomic ratio of 1.0 or greater that the gasification rate rises rapidly. In view of the data set forth in Figures 9 and 10, it can be concluded that small amounts of certain sodium compounds will catalytically activate poorly catalytic potassium sulfate; whereas greater amounts are necessary to activate poorly catalytic potassium chloride.

It will be apparent from the foregoing that the invention provides a process for gasifying a carbonaceous material which makes it possible to employ mixtures of inexpensive alkali metal salts as catalysts and at the same time attain gasification rates nearly as high as those obtainable by the use of expensive potassium carbonate. As a result, the overall cost of the product gas may be substantially reduced.

## Claims

1. A process for the catalytic gasification of a carbonaceous feed material in a reaction zone under gasification conditions in the presence of a catalyst comprising a potassium salt, wherein the process is characterized by introducing into the reaction zone: (a) a potassium salt of an organic or inorganic acid having an ionization constant exceeding 10-³ at 25°C; and (b) a sufficient quantity to activate the potassium salt of a sodium or lithium compound which is either a salt of a weak acid or a salt of a strong acid that is converted to a salt of a weak acid at the gasification conditions of the gasification process.

2. A process according to claim 1 characterized in that the carbonaceous feed material comprises coal.

3. A process according to claim 1 or claim 2 characterized in that the said carbonaceous feed material is impregnated with an aqueous solution of said potassium salt and said sodium or lithium compoud prior to the introduction of said carbonaceous feed material into said reaction zone.

4. A process according to any one of claims 1-3 characterised in that the said potassium salt comprises a salt selected from the group consisting of potassium sulfate, potassium chloride and mixtures thereof.

5. A process according to any one of claims 1-4 characterised in that the said sodium compound is selected from sodium carbonate, sodium bicarbonate, sodium sulfate, sodium hydroxide, sodium sulfide, sodium nitrate, sodium chloride (except when the potassium salt is potassium chloride) and mixtures thereof and the lithium compound is lithium sulfate.

6. A process according to any one of claims 1-5 characterised in that the said carbonaceous feed material is gasified with steam.

7. A process according to any one of claims 1-5 characterised in that the said carbonaceous feed material is gasified with hydrogen.

8. A process according to any one of claims 1-7 characterised in that said potassium salt and said sodium or lithium compounds are present in concentrations sufficient to yield a sodium or lithium to potassium atomic ratio of at least 0.25.

9. A process according to claim 8 characterized in that the potassium salt is potassium chloride and the sodium compound is present in concentrations sufficient to yield an atomic ratio of sodium to potassium of at least 1.0.

## Revendications

1. Procédé pour la gazéification catalytique d'une charbe carbonée dans une zone réactionnelle et dans des conditions de gazéification en présence d'un catalyseur . comprenant un sel de potassium, caractérisé en -ce qu'il consiste à introduire dans la zone réactionnelle: a) un sel de potassium d'un acide organique ou inorganique ayant une constante d'ionisation supérieure à 10-³ à 25°C et b) une quantité suffisante, pour activer le sel de potassium, d'un composé de sodium ou de lithium qui est un sel d'acide faible ou un sel d'acide fort qui se transforme en un sel d'un acide faible dans les conditions de gazéification du procédé de gazéification.

2. Procédé selon la revendication 1, caractérisé en ce que la charge carbonée comprend du charbon.

3. Procédé selon l'une des revendications 1 ou 2, caractérisé en ce que ladite charge carbonée est imprégnée d'une solution aqueuse dudit sel de potassium et dudit composé de sodium ou de lithium avant l'introduction de ladite charge carbonée dans la zone réactionnelle.

4. Procédé selon l'une quelconque des revendications 1 à 3, caractérisé en ce que ledit sel de potassium comprend un sel choisi dans le groupe du sulfate de potassium, du chlorure de potassium et leurs mélanges.

5. Procédé selon l'une quelconque des revendications 1 à 4, caractérisé en ce que ledit composé de sodium est choisi parmi le carbonate de sodium, le bicarbonate de sodium, le sulfate de sodium, l'hydroxyde de sodium, le sulfure de sodium, le nitrate de sodium, le chlorure de sodium (excepté lorsque le sel de potassium est le chlorure de potassium) et leurs mélanges et le composé de lithium est le sulfate de lithium.

6. Procédé selon l'une quelconque des revendications 1 à 5, caractérisé en ce que ladite charge carbonée est gazéifiée avec de la vapeur.

7. Procédé selon l'une quelconque des revendications 1 à 5, caractérisé en ce que ladite charge carbonée est gazéifiée avec de l'hydrogène.

8. Procédé selon l'une quelconque des revendications 1 à 7, caractérisé en ce que ledit sel de potassium et lesdits composés de sodium ou de lithium sont présents à des concentrations suffisantes pour fournir un rapport atomique du sodium ou du lithium au potassium d'au moins 0,25.

9. Procédé selon la revendication 8, caractérisé en ce que le sel de potassium est le chlorure de potassium et le composé de sodium est présent à des concentrations suffisantes pour fournir un rapport atomique du sodium au potassium d'au moins 1,0.

## Patentansprüche

1. Verfahren für die katalytische Vergasung von kohlenstoffhaltigem Einsatzmaterial in einer Reaktionszone unter Vergasungsbedingungen in Gegenwart eines ein Kaliumsalz enthaltenden Katalysators, dadurch gekennzeichnet, daß man in die Reaktionszone (a) ein Kaiiumsaiz einer organischen oder anorganischen Säure mit einer lonisationskonstanten größer 10-³ bei 25°C und (b) eine zur Aktivierung des Kaliumsalzes ausreichende Menge einer Natrium- oder Lithiumverbindung einbringt, wobei es sich entweder um ein Salz einer schwachen Säure oder ein Salz einer starken Säure handelt, das unter den Vergasungsbedingungen des Vergasungsverfahrens in ein Salz einer schwachen Säure umgewandelt wird.

2. Verfahren nach Anspruch 1, dadurch gekennzeichnet, daß das kohlenstoffhaltige Einsatzmaterial Kohle enthält.

3. Verfahren nach Anspruch 1 oder 2, dadurch gekennzeichnet, daß das kohlenstoffhaltige Einsatzmaterial vor dem Einbringen in die Reaktionszone mit einer wässrigen Lösung des Kaliumsalzes und der Natrium- oder Lithiumverbindung imprägniert wird.

4. Verfahren nach jedem der Ansprüche 1 bis 3, dadurch gekennzeichnet, daß das Kaliumsalz ein Salz ausgewählt aus der Gruppe bestehend aus Kaliumsulfat, Kaliumchlorid und Mischungen derselben ist.

5. Verfahren nach jedem der Ansprüche 1 bis 4, dadurch gekennzeichnet, daß die Natriumverbindung ausgewählt ist aus Natriumkarbonat, Natriumbikarbonat, Natriumsulfat, Natriumhydroxid, Natriumsulfid, Natriumnitrat, Natriumchlorid (außer wenn das Kaliumsalz Kaliumchlorid ist) und Mischungen derselben und die Lithiumverbindung Lithiumsulfat ist.

6. Verfahren nach jedem der Ansprüche 1 bis 5; dadurch gekennzeichnet, daß das kohlenstoffhaltige Einsatzmaterial mit Dampf vergast wird.

7. Verfahren nach jedem der Ansprüche 1 bis 5, dadurch gekennzeichnet, daß das kohlenstoffhaltige Einsatzmaterial mit Wasserstoff vergast wird.

8. Verfahren nach jedem der Ansprüche 1 bis 7, dadurch gekennzeichnet, daß das Kaliumsalz und die Natrium- oder Lithiumverbindungen in ausreichenden Konzentrationen vorliegen, um ein Natrium- oder Lithium/Kalium-Atomverhältnis von mindestens 0,25 zu ergeben.

9. Verfahren nach Anspruch 8, dadurch gekennzeichnet, daß das Kaliumsalz Kaliumchlorid ist und die Natriumverbindung in ausreichender Konzentration vorliegt, um ein Atomverhältnis von Natrium zu Kalium von mindestens 1,0 zu ergeben.
